



US008367286B2

(12) **United States Patent**  
**Wu**

(10) **Patent No.:** **US 8,367,286 B2**  
(45) **Date of Patent:** **Feb. 5, 2013**

(54) **PHENOLIC UREA HOLE BLOCKING LAYER  
PHOTOCONDUCTORS**

(75) Inventor: **Jin Wu**, Pittsford, NY (US)

(73) Assignee: **Xerox Corporation**, Norwalk, CT (US)

(\*) Notice: Subject to any disclaimer, the term of this patent is extended or adjusted under 35 U.S.C. 154(b) by 469 days.

(21) Appl. No.: **12/712,304**

(22) Filed: **Feb. 25, 2010**

(65) **Prior Publication Data**

US 2011/0207042 A1 Aug. 25, 2011

(51) **Int. Cl.**  
**G03G 5/14** (2006.01)

(52) **U.S. Cl.** ..... **430/65**; 430/58.8; 430/60

(58) **Field of Classification Search** ..... 430/65,  
430/58.8, 59.4, 59.5

See application file for complete search history.

(56) **References Cited**

U.S. PATENT DOCUMENTS

5,385,796 A 1/1995 Spiewak et al.  
5,449,573 A 9/1995 Aoki et al.

5,595,847 A \* 1/1997 Nogami et al. ..... 430/64  
5,928,824 A 7/1999 Obinata et al.  
6,015,645 A 1/2000 Murti et al.  
6,156,468 A 12/2000 Wehelie et al.  
6,177,219 B1 1/2001 Yuh et al.  
6,255,027 B1 7/2001 Wehelie et al.  
6,913,863 B2 7/2005 Wu et al.  
7,312,007 B2 12/2007 Lin et al.  
7,544,452 B2 6/2009 Wu et al.  
7,604,914 B2 10/2009 Lin et al.  
7,732,112 B2 \* 6/2010 Wu et al. ..... 430/60  
2009/0035673 A1 2/2009 Wu  
2009/0035674 A1 2/2009 Wu  
2009/0035675 A1 2/2009 Wu  
2009/0035676 A1 2/2009 Wu  
2009/0246668 A1 10/2009 Wu

\* cited by examiner

*Primary Examiner* — Christopher Rodee

(74) *Attorney, Agent, or Firm* — Eugene O. Palazzo

(57) **ABSTRACT**

A photoconductor that includes, for example, a substrate, an undercoat layer thereover wherein the undercoat layer contains a metal oxide dispersed in a mixture of a urea formaldehyde resin and a phenolic formaldehyde resin; a photogenerating layer; and at least one charge transport layer.

**10 Claims, No Drawings**

## 1

PHENOLIC UREA HOLE BLOCKING LAYER  
PHOTCONDUCTORSCROSS REFERENCE TO RELATED  
APPLICATIONS

Illustrated in copending U.S. application Ser. No. 12/059,536, U.S. Publication No. 20090246668, filed Mar. 31, 2008, entitled Carbazole Hole Blocking Layer Photoconductors, the disclosure of which is totally incorporated herein by reference, is a photoconductor that includes, for example, a substrate; an undercoat layer thereover wherein the undercoat layer contains a metal oxide and a carbazole containing compound; a photogenerating layer; and at least one charge transport layer.

Illustrated in copending U.S. application Ser. No. 11/831,440, U.S. Publication No. 20090035673, filed Jul. 31, 2007, entitled Iron Containing Hole Blocking Layer Containing Photoconductors, the disclosure of which is totally incorporated herein by reference, is a photoconductor comprising a substrate; an undercoat layer thereover wherein the undercoat layer comprises a metal oxide, and an iron containing compound; a photogenerating layer; and at least one charge transport layer.

Illustrated in copending U.S. application Ser. No. 11/831,453, U.S. Publication No. 20090035674, filed Jul. 31, 2007, entitled UV Absorbing Hole Blocking Layer Containing Photoconductors, the disclosure of which is totally incorporated herein by reference, is a photoconductor comprising a substrate; an undercoat layer thereover wherein the undercoat layer comprises a metal oxide, and an ultraviolet light absorber component; a photogenerating layer; and at least one charge transport layer.

Illustrated in copending U.S. application Ser. No. 11/831,476, U.S. Publication No. 20090035676, filed Jul. 31, 2007, entitled Iodonium Hole Blocking Layer Photoconductor, the disclosure of which is totally incorporated herein by reference, is a photoconductor comprising a substrate; an undercoat layer thereover wherein the undercoat layer comprises a metal oxide and an iodonium containing compound; a photogenerating layer; and at least one charge transport layer.

Illustrated in copending U.S. application Ser. No. 11/831,469, U.S. Publication No. 20090035675, filed Jul. 31, 2007, entitled Copper Containing Hole Blocking Layer Photoconductors, the disclosure of which is totally incorporated herein by reference, is a photoconductor comprising a substrate; an undercoat layer thereover wherein the undercoat layer comprises a metal oxide, and a copper containing compound; a photogenerating layer; and at least one charge transport layer.

Illustrated in copending U.S. application Ser. No. 11/211,757, U.S. Publication No. 20070049677, now U.S. Pat. No. 7,544,452, filed Aug. 26, 2005, entitled Thick Electrophotographic Imaging Member Undercoat Layers, the disclosure of which is totally incorporated herein by reference, are binders containing metal oxide nanoparticles and a co-resin of a phenolic resin and aminoplast resin, and an electrophotographic imaging member undercoat layer containing the binders.

Illustrated in copending U.S. application Ser. No. 11/403,981, U.S. Publication 20070243476, now U.S. Pat. No. 7,604,914, filed Apr. 13, 2006, entitled Imaging Members, the disclosure of which is totally incorporated herein by reference, is an electrophotographic imaging member, comprising a substrate, an undercoat layer disposed on the substrate, wherein the undercoat layer comprises a polyol resin, an aminoplast resin, and a metal oxide dispersed therein; and at least one imaging layer formed on the undercoat layer, and wherein the

## 2

polyol resin is, for example, selected from the group consisting of acrylic polyols, polyglycols, polyglycerols, and mixtures thereof.

The appropriate components and processes, number and sequence of the layers, component and component amounts in each layer, and the thicknesses of each layer of the above copending applications, may be selected for the present disclosure photoconductors in embodiments thereof.

10

## BACKGROUND

There are disclosed herein hole blocking layers, and more specifically, photoconductors containing a hole blocking layer or undercoat layer (UCL) comprised, for example, of a metal oxide, such as  $TiO_2$ , dispersed in a mixture of a urea formaldehyde resin and a phenolic formaldehyde resin, and which layer is coated or deposited on a first layer like a supporting substrate and/or a ground plane layer of, for example, aluminum, titanium, zirconium, gold, or a gold containing compound.

In embodiments, photoconductors comprised of the disclosed hole blocking or undercoat layer enables, for example, the blocking of or minimization of the movement of holes or positive charges generated from the ground plane layer, and excellent cyclic stability, and thus color print stability especially for xerographic generated color copies. Excellent cyclic stability of the photoconductor refers, for example, to almost no or minimal change in a generated known photoinduced discharge curve (PIDC), especially no or minimal residual potential cycle up after a number of charge/discharge cycles of the photoconductor, for example about 200 kilocycles, or xerographic prints of, for example, from about 75 to about 250 kiloprints. Excellent color print stability refers, for example, to substantially no or minimal change in solid area density, especially in 50 to 60 percent halftone prints, and no or minimal random color variability from print to print after a number of xerographic prints, for example 70 kiloprints.

Further, in embodiments the photoconductors disclosed permit the minimization or substantial elimination of undesirable ghosting on developed images, such as xerographic images, including minimal ghosting, especially as compared to a similar photoconductor where the resin mixture disclosed herein is absent and at various relative humidities; excellent cyclic and stable electrical properties; acceptable charge deficient spots (CDS); and compatibility with the photogenerating and charge transport resin binders, such as polycarbonates. Charge blocking layer and hole blocking layer are generally used interchangeably with the phrase "undercoat layer".

The need for excellent print quality in xerographic systems is of value, especially with the advent of color. Common print quality issues can be dependent on the components of the undercoat layer (UCL). When the undercoat layer is too thin, then incomplete coverage of the substrate may sometimes result due to wetting problems on localized unclean substrate surface areas. This incomplete coverage may produce pin holes which can, in turn, produce print defects such as charge deficient spots (CDS) and bias charge roll (BCR) leakage breakdown. Other problems include image "ghosting" resulting from, it is believed, the accumulation of charge somewhere in the photoreceptor. Removing trapped electrons and holes residing in the imaging members is a factor in preventing ghosting. During the exposure and development stages of xerographic cycles, the trapped electrons are mainly at or near the interface between the charge generation layer (CGL) and the undercoat layer (UCL), and holes are present mainly at or near the interface between the charge generation layer and the

charge transport layer (CTL). The trapped charges can migrate according to the electric field during the transfer stage where the electrons can move from the interface of CGL/UCL to CTL/CGL, or the holes from CTL/CGL to CGL/UCL, and become deep traps that are no longer mobile. Consequently, when a sequential image is printed, the accumulated charge results in image density changes in the current printed image that reveals the previously printed image. Thus, there is a need to minimize or eliminate charge accumulation in photoreceptors without sacrificing the desired thickness of the undercoat layer, and a need for permitting the UCL to properly adhere to the other photoconductive layers, such as the photogenerating layer, for extended time periods, such as for example, about 750,000 simulated xerographic imaging cycles. Thus, a number of conventional materials used for the undercoat or blocking layer possess a number of disadvantages resulting in adverse print quality characteristics. For example, ghosting, charge deficient spots, and bias charge roll leakage breakdown are problems that commonly occur and which problems are minimized with the photoconductors illustrated herein.

Thick undercoat layers are sometimes desirable for xerographic photoconductors as such layers permit photoconductor life extension and carbon fiber resistance. Furthermore, thicker undercoat layers permit the use of economical substrates in the photoreceptors. Examples of thick undercoat layers are disclosed in U.S. Pat. No. 7,312,007, however, due primarily to insufficient electron conductivity in dry and cold environments, the residual potential in conditions, such as 10 percent relative humidity and 70° F., can be high when the undercoat layer is thicker than about 15 microns, and moreover, the adhesion of the UCL may be poor, disadvantages avoided or minimized with the UCL of the present disclosure.

Also included within the scope of the present disclosure are methods of imaging and printing with the photoconductive devices illustrated herein. These methods generally involve the formation of an electrostatic latent image on the imaging member, followed by developing the image with a toner composition comprised, for example, of a thermoplastic resin, colorant, such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, the imaging members, photoconductor drums, and flexible belts disclosed herein can be selected for the Xerox Corporation iGEN3® machines that generate with some versions over 100 copies per minute. Processes of imaging, especially xerographic imaging and printing, including digital, and/or high speed color printing, are thus encompassed by the present disclosure.

The photoconductors disclosed herein are, in embodiments, sensitive in the wavelength region of, for example, from about 400 to about 900 nanometers, and in particular from about 650 to about 850 nanometers, thus diode lasers can be selected as the light source.

#### REFERENCES

Illustrated in U.S. Pat. No. 6,913,863 is a photoconductive imaging member comprised of an optional supporting substrate, a hole blocking layer thereover, a photogenerating layer, and a charge transport layer, and wherein the hole

blocking layer is comprised of a metal oxide, and a mixture of phenolic resins, and wherein at least one of the resins contains two hydroxy groups.

Illustrated in U.S. Pat. Nos. 6,255,027; 6,177,219, and 6,156,468, are, for example, photoreceptors containing a charge blocking layer of a plurality of light scattering particles dispersed in a binder, reference for example, Example I of U.S. Pat. No. 6,156,468, wherein there is illustrated a charge blocking layer of titanium dioxide dispersed in a specific linear phenolic binder of VARCUM®, available from OxyChem Company.

Illustrated in U.S. Pat. No. 6,015,645 is a photoconductive imaging member comprised of a supporting substrate, a hole blocking layer, an optional adhesive layer, a photogenerating layer, and a charge transport layer, and wherein the blocking layer is comprised of a polyhaloalkylstyrene.

Illustrated in U.S. Pat. No. 5,473,064, the disclosure of which is totally incorporated herein by reference, is a process for the preparation of hydroxygallium phthalocyanine Type V, essentially free of chlorine.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photogenerating pigments, which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water, concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

A number of photoconductors are disclosed in U.S. Pat. No. 5,489,496; U.S. Pat. No. 4,579,801; U.S. Pat. No. 4,518,669; U.S. Pat. No. 4,775,605; U.S. Pat. No. 5,656,407; U.S. Pat. No. 5,641,599; U.S. Pat. No. 5,344,734; U.S. Pat. No. 5,721,080; and U.S. Pat. No. 5,017,449, U.S. Pat. No. 6,200,716; U.S. Pat. No. 6,180,309; and U.S. Pat. No. 6,207,334.

A number of undercoat or charge blocking layers are disclosed in U.S. Pat. No. 4,464,450; U.S. Pat. No. 5,449,573; U.S. Pat. No. 5,385,796; and U.S. Pat. No. 5,928,824.

#### SUMMARY

According to embodiments illustrated herein, and wherein ghosting is minimized or substantially eliminated, in images printed with, for example, xerographic imaging systems, there are provided photoconductors that enable, it is believed, acceptable print quality in systems with high transfer current and improved CDS characteristics as compared, for example, to a similar photoconductor where the resin mixture illustrated herein is absent.

Embodiments disclosed herein also include a photoconductor comprising a substrate, a ground plane layer, and an undercoat layer as illustrated herein, disposed, or deposited on the ground plane layer, a photogenerating layer, and a

charge transport layer formed on the photogenerating layer; a photoconductor comprised of a substrate, a ground plane layer, an undercoat layer disposed on the ground plane, wherein the undercoat layer comprises a metal oxide, such as  $\text{TiO}_2$ , dispersed in a mixture of a urea formaldehyde resin and a phenolic formaldehyde resin mixture, and which photoconductors exhibited excellent electrical characteristics at time zero ( $t=0$  PIDC) and cyclic stability, low background, and excellent ghosting properties, and which undercoat layer primarily functions to provide for blocking holes from the supporting substrate, and excellent cyclic stability for the photoconductor, thus color stability for the xerographic prints.

## EMBODIMENTS

Aspects of the present disclosure relate to a photoconductor comprising a photoconductor comprising a substrate, an undercoat layer thereover wherein the undercoat layer comprises a metal oxide, and a mixture of a urea formaldehyde resin and a phenolic formaldehyde resin; a photogenerating layer; and a charge transport layer; a photoconductor comprising a supporting substrate; an undercoat layer thereover comprised of a mixture of a metal oxide, a urea formaldehyde polymer and a phenolic formaldehyde polymer; a photogenerating layer, and a charge transport layer, and wherein the resin mixture forms a crosslinked polymeric network; a photoconductor comprising in sequence a supporting substrate, an undercoat layer thereover comprised of a crosslinked interpolymer network mixture of a metal oxide, a urea formaldehyde resin and a phenolic formaldehyde resin; a photogenerating layer, and a hole transport layer; the phenolic formaldehyde resin is selected from the group consisting of a phenol formaldehyde, a p-tert-butylphenol formaldehyde and a cresol formaldehyde resin, a 4,4'-(1-methylethylidene) bisphenol formaldehyde resin, a resin generated from a phenol and cresol formaldehyde resin, or a resin generated from a phenol and p-tert-butylphenol formaldehyde resin; the metal oxide is selected from the group consisting of titanium oxide, zinc oxide, tin oxide, aluminum oxide, silicone oxide, zirconium oxide, indium oxide, and molybdenum oxide; the photogenerating layer is comprised of a pigment and a resin binder; the hole transport layer is comprised of aryl amine molecules and a resin binder; and wherein the crosslinking value is from about 40 to about 90 percent, and wherein the urea formaldehyde resin comprises urea formaldehyde moieties represented by the following formula/structure



wherein  $R_1$ ,  $R_2$ ,  $R_3$  and  $R_4$  are at least one of alkyl, and a hydrogen atom, and  $w$ ,  $x$ ,  $y$  and  $z$  each independently a number, such as 0 or 1; a photoconductor comprising a substrate, an optional ground plane layer, an undercoat layer thereover wherein the undercoat layer comprises metal oxide dispersed in a mixture of a urea formaldehyde resin and a phenolic formaldehyde resin, a photogenerating layer and at least one charge transport layer; a photoconductor comprising a substrate; a ground plane layer, an undercoat or hole blocking

layer thereover comprised of a mixture of metal oxide, a urea formaldehyde resin and a phenolic formaldehyde resin, a photogenerating layer, and a charge transport layer; a rigid drum or flexible belt photoconductor comprising in sequence 5 a supporting substrate, a ground plane layer, a hole blocking layer comprised of metal oxide dispersed in a mixture of a urea formaldehyde resin and a phenolic formaldehyde resin, a photogenerating layer, and a charge transport layer, and wherein the phenolic formaldehyde resin is commercially 10 available from a number of sources and can be formed, for example, by the reaction of an aldehyde and a phenol source in the presence of an acidic or basic catalyst; a photoconductor comprising a supporting substrate, an undercoat layer thereover wherein the undercoat layer comprises a metal 15 oxide such as a titanium oxide, a zinc oxide, an antimony tin oxide, and other known suitable oxides, dispersed in a mixture of a urea formaldehyde resin and a phenolic formaldehyde resin, and which mixture contains, for example, from 1 to about 99 percent by weight of the urea formaldehyde resin 20 or polymer, and from about 99 to about 1 weight percent of the phenolic formaldehyde resin or polymer, a photogenerating layer, and at least one charge transport layer, where at least one is, for example, from 1 to about 7, from 1 to about 5, from 1 to about 3, 1, or 2 layers; a photoconductor comprising a 25 supporting substrate, an undercoat layer thereover comprised of a mixture of a metal oxide or metal oxides contained in a mixture of urea formaldehyde resins and phenolic formaldehyde resins, a photogenerating layer, and a charge transport layer; a rigid drum or flexible belt photoconductor comprising in sequence a supporting substrate, such as a nonconductive substrate, thereover an optional ground plane layer; a hole blocking layer comprised of a metal oxide dispersed in a mixture of a urea formaldehyde resin and a phenolic formaldehyde resin, thereover a photogenerating layer, and a charge 30 transport layer; a photoconductive member or device comprising a substrate, a ground plane layer, the robust undercoat layer illustrated herein, and at least one imaging layer, such as a photogenerating layer and a charge transport layer or layers, formed on the undercoat layer; a photoconductor wherein the 35 photogenerating layer is situated between the charge transport layer and the substrate, and which layer contains a resin binder; an electrophotographic imaging member, which generally comprises at least a substrate layer, a ground plane layer, an undercoat layer, and deposited on the undercoat 40 layer in sequence a photogenerating layer and a charge transport layer; a photoconductor wherein the photogenerating layer is situated between the charge transport layer and the substrate, and which layer contains a resin binder; an electrophotographic imaging member, which generally comprises at least a substrate layer, a ground plane layer, an undercoat layer, and deposited on the undercoat 45 layer in sequence a photogenerating layer and a charge transport layer.

## Undercoat Layer Component Examples

50 In embodiments, the phenolic resin or resins that may be selected for the preparation of the phenolic formaldehyde resin in various effective amounts, such as from about 1 to about 60 weight percent, from about 5 to about 40 weight percent, from about 10 to about 30 weight percent, and more 55 specifically, about 20 weight percent, can be considered to be formed by the condensation product of an aldehyde with a phenol source in the presence of an acidic or basic catalyst. The phenol source may be, for example, phenol; alkyl-substituted phenols, such as cresols and xylenols; halogen-substituted phenols, such as chlorophenol; polyhydric phenols, such as resorcinol or pyrocatechol; polycyclic phenols, such as naphthol and bisphenol A; aryl-substituted phenols, cycloalkyl-substituted phenols, aryloxy-substituted phenols, and various mixtures thereof. Examples of a number of phenol 60 sources are 2,6-xylenol, o-cresol, p-cresol, 3,5-xylenol, 3,4-xylenol, 2,3,4-trimethyl phenol, 3-ethyl phenol, 3,5-diethyl phenol, p-butyl phenol, 3,5-dibutyl phenol, p-amyl phenol, 65

p-cyclohexyl phenol, p-octyl phenol, 3,5-dicyclohexyl phenol, p-phenyl phenol, p-crotyl phenol, 3,5-dimethoxy phenol, 3,4,5-trimethoxy phenol, p-ethoxy phenol, p-butoxy phenol, 3-methyl-4-methoxy phenol, p-phenoxy phenol, multiple ring phenols, such as bisphenol A, and combinations thereof. The aldehyde may be, for example, formaldehyde, paraformaldehyde, acetaldehyde, butyraldehyde, paraldehyde, glyoxal, furfuraldehyde, propinonaldehyde, benzaldehyde, and various mixtures thereof, and the phenolic resin selected for the hole blocking or undercoat layer may be, for example, dicyclopentadiene type phenolic resins; phenol Novolak resins; cresol Novolak resins; phenol aralkyl resins; and mixtures thereof; formaldehyde polymers with phenol, p-tert-butylphenol, and cresol, such as VARCUM™ 29159 and 29101 (available from OxyChem Company), and DURITE™ 97 (available from Borden Chemical); formaldehyde polymers with ammonia, cresol, and phenol (available from OxyChem Company); formaldehyde polymers with 4,4'-(1-methyl ethylidene)bisphenol, such as VARCUM™ 29108 and 29116 (available OxyChem Company); formaldehyde polymers with cresol and phenol, such as VARCUM™ 29457 (available from OxyChem Company); DURITE™ SD-423A, SD-422A (Borden Chemical); formaldehyde polymers with phenol and p-tert-butylphenol, such as DURITE™ ESD 556C (available from Borden Chemical); mixtures thereof, and a number of suitable known phenolic resins.

In embodiments, the phenolic resins selected are base-catalyzed phenol formaldehyde resins that are generated with a formaldehyde/phenol mole ratio of equal to or greater than one, for example, from about 1 to about 2; or from about 1.2 to about 1.8; or about 1.5. The base catalyst, such as an amine, is generally miscible with the phenol resin.

Examples of the urea formaldehyde resin include a number of known resins as illustrated herein, and more specifically, comprising urea formaldehyde moieties represented by



wherein  $R_1$ ,  $R_2$ ,  $R_3$  and  $R_4$  are at least one of alkyl, and a hydrogen atom wherein alkyl, for example, contains 1 to about 18, 1 to about 12, 1 to about 8, 1 to about 6 and from 1 to about 46 carbon atoms, and  $w$ ,  $x$ ,  $y$  and  $z$  each independently represents the number of groups or segments, and is, for example, 0 or 1, and which urea resin can be water soluble, dispersible, or indispersible. The urea resin selected in 55 embodiments is highly alkylated/alkoxylated, partially alkylated/alkoxylated, or mixed alkylated/alkoxylated, and more specifically, the urea resin is a methylated, n-butylated, or isobutylated polymer. Specific examples of the urea resin include methylated urea resins such as CYMEL® U-65, 60 UM-15, U-382; n-butylated urea resins such as CYMEL® U-80, U-1054, UB-30-B ( $M_w=10,000$ ), UB-24-BX ( $M_w=6,000$ ), UB-25-BE ( $M_w=5,000$ ), UB-26-BX ( $M_w=6,000$ ), UB-90-BX ( $M_w=3,000$ ), U-227-8 ( $M_w=6,000$ ), U-610 ( $M_w=4,000$ ), U-640 ( $M_w=2,500$ ); or isobutylated urea resins 65 such as CYMEL® U-662 ( $M_w=4,000$ ), U-646 ( $M_w=4,000$ ), U-663 ( $M_w=4,000$ ), U-665 ( $M_w=4,000$ ), UI-19-I ( $M_w=6,$

000), UI-19-IE ( $M_w$ =6,000), UI-20-E ( $M_w$ =2,000), UI-38-I ( $M_w$ =4,000). CYMEL® urea resins are commercially available from CYTEC Industries.

In embodiments, the urea formaldehyde resin possess a number average molecular weight of from about 200 to about 8,000, or from about 800 to about 4,000; a weight average molecular weight of from about 300 to about 10,000, or from about 1,000 to about 6,000, as determined by Gel Permeation Chromatography (GPC).

10 Examples of specific urea formaldehyde resins are urea formaldehyde moieties represented by at least one of



Various amounts of the metal oxide and the resin mixture can be selected for the undercoat layer. For example from about 1 to about 99 weight percent, from about 10 to about 75 weight percent, or from about 25 to about 50 weight percent of the urea formaldehyde resin can be selected, and from about 99 to about 1 weight percent, from about 90 to about 25 weight percent, or from about 75 to about 50 weight percent of the phenolic formaldehyde resin polymeric binder can be selected, and where the total of the two resins in the mixture amount to about 100 percent.

The hole blocking layer thickness can be of any suitable value, such as for example, from about 0.1 to about 30 microns, from about 1 to about 20 microns, or from about 3 to about 15 microns.

In embodiments, the undercoat layer metal oxide like  $TiO_2$  can be either surface treated or untreated. Surface treatments include, but are not limited to, mixing the metal oxide with aluminum laurate, alumina, zirconia, silica, silane, methicone, dimethicone, sodium metaphosphate, and the like, and mixtures thereof. Examples of  $TiO_2$  include MT-150W<sup>TM</sup> (surface treatment with sodium metaphosphate, available from Tayca Corporation), STR-60N<sup>TM</sup> (no surface treatment, available from Sakai Chemical Industry Co., Ltd.), FTL-100<sup>TM</sup> (no surface treatment, available from Ishihara Sangyo Laisha, Ltd.), STR-60<sup>TM</sup> (surface treatment with  $Al_2O_3$ , available from Sakai Chemical Industry Co., Ltd.), TTO-55N<sup>TM</sup> (no surface treatment, available from Ishihara Sangyo Laisha, Ltd.), TTO-55A<sup>TM</sup> (surface treatment with  $Al_2O_3$ , available from Ishihara Sangyo Laisha, Ltd.), MT-150AW<sup>TM</sup> (no surface treatment, available from Tayca Corporation), MT-150A<sup>TM</sup> (no surface treatment, available from Tayca Corporation), MT-100S<sup>TM</sup> (surface treatment with aluminum laurate and alumina, available from Tayca Corporation), MT-100HD<sup>TM</sup> (surface treatment with zirconia and alumina, available from Tayca Corporation), MT-100SA<sup>TM</sup> (surface treatment with silica and alumina, available from Tayca Corporation), and the like.

Examples of metal oxides present in suitable amounts, such as for example, from about 5 to about 80 weight percent, and more specifically, from about 30 to about 70 weight percent, are titanium oxides and mixtures of metal oxides thereof. In embodiments, the metal oxide has a size diameter of from about 5 to about 300 nanometers, a powder resistance of from about  $1 \times 10^3$  to about  $6 \times 10^5$  ohm/cm when applied at a pressure of from about 50 to about 650 kilograms/cm<sup>2</sup>, and yet more specifically, the titanium oxide possesses a primary particle size diameter of from about 10 to about 25 nanometers, and more specifically, from about 12 to about 17 nanometers, and yet more specifically, about 15 nanometers with an estimated aspect ratio of from about 4 to about 5, and is optionally surface treated with, for example, a component containing, for example, from about 1 to about 3 percent by weight of alkali metal, such as a sodium metaphosphate, a powder resistance of from about  $1 \times 10^4$  to about  $6 \times 10^4$  ohm/cm when applied at a pressure of from about 650 to about 50 kilograms/cm<sup>2</sup>; MT-150W<sup>TM</sup>, and which titanium oxide is available from Tayca Corporation, and wherein the hole blocking layer is of a suitable thickness, such as a thickness of about from about 0.1 to about 30 microns, thereby avoiding or minimizing charge leakage. Metal oxide examples in addition to titanium are chromium, zinc, tin, copper, antimony, and the like, and more specifically, zinc oxide, tin oxide, aluminum oxide, silicone oxide, zirconium oxide, indium oxide, molybdenum oxide, and mixtures thereof.

The hole blocking layer can, in embodiments, be prepared by a number of known methods, the process parameters being dependent, for example, on the photoconductor member desired. The hole blocking layer can be coated as a solution or a dispersion onto the ground plane layer by the use of a spray coater, dip coater, extrusion coater, roller coater, wire-bar coater, slot coater, doctor blade coater, gravure coater, and the like, and dried at from about 40° C. to about 200° C. for a suitable period of time, such as from about 1 minute to about 10 hours, under stationary conditions or in an air flow. The coating can be accomplished to provide a final coating thick-

ness of from about 0.1 to about 30 microns, or from about 1 to about 20 microns, or from about 3 to about 15 microns, after drying.

#### Photoconductor Layer Examples

The layers of the photoconductor, in addition to the undercoat layer, can be comprised of a number of known layers, such as supporting substrates, adhesive layers, photogenerating layers, charge transport layers and protective overcoating top layers, such as the examples of these layers as illustrated in the copending applications referenced herein.

The thickness of the photoconductive substrate layer depends on many factors including economical considerations, electrical characteristics, and the like; thus, this layer may be of a substantial thickness, for example in excess of 3,000 microns, such as from about 500 to about 2,000 microns, from about 300 to about 700 microns, or of a minimum thickness. In embodiments, the thickness of this layer is from about 75 to about 275 microns, or from about 95 to about 140 microns.

The substrate may be opaque, substantially transparent, or be of a number of other suitable known forms, and may comprise any suitable material having the required mechanical properties. Accordingly, the substrate may comprise a layer of an electrically nonconductive or conductive material such as an inorganic or an organic composition. As electrically nonconducting materials, there may be employed various resins known for this purpose including polyesters, poly-carbonates, polyamides, polyurethanes, and the like, which are flexible as thin webs. An electrically conducting substrate may be any suitable metal of, for example, aluminum, nickel, steel, copper, and the like, or a polymeric material, as described above, filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like. The thickness of the substrate layer depends on numerous factors including strength desired and economical considerations. For a drum, as disclosed in a copending application referenced herein, this layer may be of a substantial thickness of, for example, up to many centimeters or of a minimum thickness of less than a millimeter. Similarly, a flexible belt may be of a substantial thickness of, for example, about 250 microns, or of a minimum thickness of less than about 50 microns, provided there are no adverse effects on the final electrophotographic device. In embodiments, where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, substrates selected for the imaging members of the present disclosure, and which substrates can be opaque or substantially transparent comprise a layer of insulating material including inorganic or organic polymeric materials, such as MYLAR<sup>®</sup> a commercially available polymer, MYLAR<sup>®</sup> containing titanium, a layer of an organic or inorganic material having a semiconductive surface layer, such as indium tin oxide, or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In

## 11

embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

The photogenerating layer in embodiments is comprised of, for example, a number of known photogenerating pigments including, for example, Type V hydroxygallium phthalocyanine, Type IV or V titanyl phthalocyanine, or chlorogallium phthalocyanine, and a resin binder like poly(vinyl chloride-co-vinyl acetate) copolymer, such as VMCH (available from Dow Chemical), or polycarbonate. Generally, the photogenerating layer can contain known photogenerating pigments, such as metal phthalocyanines, metal free phthalocyanines, alkylhydroxygallium phthalocyanines, hydroxygallium phthalocyanines, chlorogallium phthalocyanines, perylenes, especially bis(benzimidazo)perylene, titanyl phthalocyanines, and the like, and more specifically, vanadyl phthalocyanines, Type V hydroxygallium phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount of photogenerating material contained in the photogenerating layer. Accordingly, this layer can be of a thickness of, for example, from about 0.05 to about 10 microns, and more specifically, from about 0.25 to about 2 microns when, for example, the photogenerating compositions are present in an amount of from about 30 to about 75 percent by volume. The maximum thickness of this layer, in embodiments, is dependent primarily upon factors, such as photosensitivity, electrical properties, and mechanical considerations. The photogenerating layer binder resin is present in various suitable amounts of, for example, from about 1 to about 50 weight percent, and more specifically, from about 1 to about 10 weight percent, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Generally, however, from about 5 to about 90 percent by volume of the photogenerating pigment is dispersed in about 10 to about 95 percent by volume of the resinous binder, or from about 20 to about 30 percent by volume of the photogenerating pigment is dispersed in about 70 to about 80 percent by volume of the resinous binder composition. In one embodiment, about 8 percent by volume of the photogenerating pigment is dispersed in about 92 percent by volume of the resinous binder composition. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

## 12

The photogenerating layer may comprise amorphous films of selenium and alloys of selenium and arsenic, tellurium, germanium, and the like, hydrogenated amorphous silicone and compounds of silicone and germanium, carbon, oxygen, nitrogen, and the like fabricated by vacuum evaporation or deposition. The photogenerating layer may also comprise inorganic pigments of crystalline selenium and its alloys; Groups II to VI compounds; and organic pigments such as quinacridones; polycyclic pigments such as dibromoanthranthrone pigments, perylene and perinone diamines; polynuclear aromatic quinones, azo pigments including bis-, tris- and tetrakis-azos, and the like dispersed in a film forming polymeric binder and fabricated by solvent coating techniques.

Examples of polymeric binder materials that can be selected as the matrix for the photogenerating layer components are thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly(vinyl chloride), vinyl chloride and vinyl acetate copolymers, acrylate copolymers, alkyd resins, cellulosic film formers, poly(amideimide), styrenebutadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

Various suitable and conventional known processes may be selected to mix, and thereafter apply the photogenerating layer coating mixture to the substrate, and more specifically, to the hole blocking layer or other layers like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like. The coating of the photogenerating layer on the UCL (undercoat layer) in embodiments of the present disclosure can be accomplished such that the final dry thickness of the photogenerating layer is as illustrated herein, and can be, for example, from about 0.01 to about 30 microns after being dried at, for example, about 40° C. to about 150° C. for about 1 to about 90 minutes. More specifically, a photogenerating layer of a thickness, for example, of from about 0.1 to about 30 microns, or from about 0.5 to about 2 microns can be applied to or deposited on the substrate, on other surfaces in between the substrate and the charge transport layer, and the like. The hole blocking layer or UCL may be applied to the ground plane layer prior to the application of a photogenerating layer.

A suitable known adhesive layer can be included in the photoconductor. Typical adhesive layer materials include, for example, polyesters, polyurethanes, and the like. The adhesive layer thickness can vary, and in embodiments is, for example, from about 0.05 to about 0.3 micron. The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like. As optional adhesive layers usually in contact with or situated

between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicone nitride, carbon black, and the like, to provide, for example, in embodiments of the present disclosure, further desirable electrical and optical properties.

A number of charge transport materials, especially known hole transport molecules, and polymers may be selected for the charge transport layer, examples of which are aryl amines of the formulas/structures



and which layer is generally of a thickness of from about 5 to about 75 microns, and more specifically, of a thickness of from about 10 to about 40 microns, wherein X is a suitable hydrocarbon like alkyl, alkoxy, and aryl, a halogen, or mixtures thereof, and especially those substituents selected from the group consisting of Cl and CH<sub>3</sub>; and molecules of the following formulas



wherein X, Y and Z are a suitable substituent like a hydrocarbon, such as independently alkyl, alkoxy, or aryl, a halogen, or mixtures thereof, and wherein at least one of Y or Z is present. Alkyl and alkoxy contain, for example, from 1 to about 25 carbon atoms, from 1 to about 18 carbon atoms, from 1 to about 12 carbon atoms, and more specifically, from 1 to about 6 carbon atoms, and from 1 to about 4 carbon atoms, such as methyl, ethyl, propyl, butyl, pentyl, and the corresponding alkoxides. Aryl can contain from 6 to about 42

carbon atoms, from 6 to about 36 carbon atoms, from 6 to about 24 carbon atoms, from 6 to about 18 carbon atoms, such as phenyl, and the like. Halogen includes chloride, bromide, iodide, and fluoride. Substituted alkyls, alkoxy, and aryls can also be selected in embodiments. At least one charge transport refers, for example, to 1, from 1 to about 7, from 1 to about 4, and from 1 to about 2.

Examples of specific aryl amines include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4"-diamine, N,N'-bis(4-butylphenyl)-N,N-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine, and the like. Other known charge transport layer molecules can be selected, reference for example, U.S. Pat. Nos. 4,921,773 and 4,464,450, the disclosures of which are totally incorporated herein by reference.

Examples of the binder materials selected for the charge transport layer or layers include polycarbonates, polyarylates, acrylate polymers, vinyl polymers, cellulose polymers, polyesters, polysiloxanes, polyamides, polyurethanes, poly(cyclo olefins), epoxies, and random or alternating copolymers thereof; and more specifically, polycarbonates such as poly(4,4'-isopropylidene-diphenylene)carbonate (also referred to as bisphenol-A-polycarbonate), poly(4,4'-cyclohexylidene diphenylene)carbonate (also referred to as bisphenol-Z-polycarbonate), poly(4,4'-isopropylidene-3,3'-dimethyl-diphenyl)carbonate (also referred to as bisphenol-C-polycarbonate), and the like. In embodiments, electrically inactive binders are comprised of polycarbonate resins with a molecular weight of from about 20,000 to about 100,000, or with a molecular weight M<sub>w</sub> of from about 50,000 to about 100,000 preferred. Generally, the transport layer contains from about 10 to about 75 percent by weight of the charge transport material, and more specifically, from about 35 percent to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules selected for the charge transport layer or layers, and present in various effective amounts include, for example, pyrazolines such as 1-phenyl-3-(4'-diethylamino styryl)-5-(4"-diethylamino phenyl)

15

pyrazoline; aryl amines such as N,N'-diphenyl-N,N'-bis(3-methylphenyl)-(1,1'-biphenyl)-4,4'-diamine, tetra-p-tolyl-biphenyl-4,4'-diamine, N,N'-diphenyl-N,N'-bis(4-methoxyphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-diphenyl-N,N'-bis(3-chlorophenyl)-[p-terphenyl]-4,4"-diamine; hydrazones such as N-phenyl-N-methyl-3-(9-ethyl)carbazyl hydrazone, and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like. A small molecule charge transporting compound that permits injection of holes into the photogenerating layer with high efficiency, and transports them across the charge trans-

16

port layer with short transit times includes N,N'-diphenyl-N,N'-bis(3-methylphenyl)-(1,1'-biphenyl)-4,4'-diamine, tetra-p-tolyl-biphenyl-4,4'-diamine, N,N'-diphenyl-N,N'-bis(4-methoxyphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-diphenyl-N,N'-bis(3-chlorophenyl)-[p-terphenyl]-4,4"-diamine, or mixtures thereof. If desired, the charge transport material in the charge transport layer may comprise a polymeric charge transport material or a combination of a small molecule charge transport material and a polymeric charge transport material.

In embodiments, the charge transport component can be represented by the following formulas/structures



and



-continued



Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate) methane (IRGANOX™ 1010, available from Ciba Specialty Chemical), butylated hydroxytoluene (BHT), and other hindered phenolic antioxidants including SUMILIZER™ BHT-R, MDP-S, BBM-S, WX-R, NR, BP-76, BP-101, GA-80, GM and GS (available from Sumitomo Chemical Co., Ltd.), IRGANOX™ 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Co., Ltd.); hindered amine antioxidants such as SANOL™ LS-2626, LS-765, LS-770 and LS-744 (available from SNKYO CO., Ltd.), TINUVIN™ 144 and 622LD (available from Ciba Specialties Chemicals), MARK™ LA57, LA67, LA62, LA68 and LA63 (available from Asahi Denka Co., Ltd.), and SUMILIZER™ TPS (available from Sumitomo Chemical Co., Ltd.); thioether antioxidants such as SUMILIZER™ TP-D (available from Sumitomo Chemical Co., Ltd.); phosphite antioxidants such as MARK™ 2112, PEP-8, PEP-24G, PEP-36, 329K and HP-10 (available from Asahi Denka Co., Ltd.); other molecules such as bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20 weight percent, from about 1 to about 10 weight percent, or from about 3 to about 8 weight percent.

A number of processes may be used to mix, and thereafter apply the charge transport layer or layers coating mixture to the photogenerating layer. Typical application techniques include spraying, dip coating, and roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is, for example, from about 10 to about 75 microns, from about 15 to about 50 microns, but thicknesses outside these ranges may, in embodiments, also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thick-

ness of the charge transport layer to the photogenerating layer can be from about 2:1 to about 200:1, and in some instances 20 400:1. The charge transport layer is substantially nonabsorbing to visible light or radiation in the region of intended use, but is electrically "active" in that it allows the injection of photogenerated holes from the photoconductive layer or photogenerating layer, and allows these holes to be transported 25 through itself to selectively discharge a surface charge on the surface of the active layer.

The thickness of the continuous charge transport layer selected depends upon the abrasiveness of the charging (bias charging roll), cleaning (blade or web), development (brush), 30 transfer (bias transfer roll), and the like in the system employed, and can be up to about 10 microns. In embodiments, the thickness for each charge transport layer can be, for example, from about 1 to about 5 microns. Various suitable and conventional methods may be used to mix, and thereafter apply an overcoat top charge transport layer coating mixture to the photoconductor. Typical application techniques include spraying, dip coating, roll coating, wire wound rod coating, and the like. Drying of the deposited coating may 35 be effected by any suitable conventional technique, such as oven drying, infrared radiation drying, air drying, and the like. The dried overcoat layer of this disclosure should transport holes during imaging, and should not have too high a free carrier concentration. Free carrier concentration in the overcoat increases the dark decay.  $M_w$ , weight average molecular weight, and  $M_n$ , number average molecular weight, were 40 determined by Gel Permeation Chromatography.

The following Examples are provided. All proportions are 45 by weight unless otherwise indicated.

#### Comparative Example 1

A dispersion of a hole blocking layer was prepared by 50 milling 18 grams of  $TiO_2$  (MT-150W, manufactured by Tayca Co., Japan), and 24 grams of the phenolic resin (VARCUM™ 29159, OxyChem Co., about 50 percent in xylene/1-butanol=50/50) in a solvent mixture of xylene and 1-butanol 55 (50/50 mixture), and a total solid content of about 48 percent in an attritor mill with about 0.4 to about 0.6 millimeter size  $ZrO_2$  beads for 6.5 hours, and then filtering with a 20 micron 60  $Nylon$  filter. A 30 millimeter aluminum drum substrate was then coated with the aforementioned generated dispersion using known coating techniques as illustrated herein. After drying at 160°C. for 20 minutes, a hole blocking layer of  $TiO_2$  in the phenolic resin ( $TiO_2$ /phenolic resin=60/40) about 6 65 microns in thickness was obtained.

A photogenerating layer comprising chlorogallium phthalocyanine was deposited on the above hole blocking layer or

19

undercoat layer at a thickness of about 0.2 micron. The photogenerating layer coating dispersion was prepared as follows. 2.7 Grams of chlorogallium phthalocyanine (ClGaPc) Type C pigment were mixed with 2.3 grams of the polymeric binder (carboxyl modified vinyl copolymer, VMCH, Dow Chemical Company), 15 grams of n-butyl acetate, and 30 grams of xylene. The resulting mixture was milled in an attritor mill with about 200 grams of 1 millimeter Hi-Bea borosilicate glass beads for about 3 hours. The dispersion mixture obtained was then filtered through a 20 micron Nylon cloth filter, and the solids content of the dispersion was diluted to about 6 weight percent.

Subsequently, a 30 micron thick charge transport layer was coated on top of the photogenerating layer from a dispersion prepared from N,N'-diphenyl-N,N-bis(3-methylphenyl)-1,1'-biphenyl-4,4'-diamine (5.38 grams), a film forming polymer binder, PCZ-400 [poly(4,4'-dihydroxy-diphenyl-1-1-cyclohexane,  $M_w=40,000$ )] available from Mitsubishi Gas Chemical Company, Ltd. (7.13 grams), and PTFE POLY-FLONTM L-2 microparticle (1 gram), available from Daikin Industries, dissolved/dispersed in a solvent mixture of 20 grams of tetrahydrofuran (THF), and 6.7 grams of toluene through a CAVIPROTM 300 nanomizer (Five Star Technology, Cleveland, Ohio). The charge transport layer was dried at about 120° C. for about 40 minutes.

#### Example I

A photoconductor was prepared by repeating the above process of Comparative Example 1, except that the hole blocking layer dispersion was prepared by milling 18 grams of  $TiO_2$  (MT-150W, manufactured by Tayca Co., Japan), 9.6 grams of the phenolic formaldehyde resin VARCUMTM 29159 (obtained from OxyChem Company, about 50 percent in xylene/1-butanol=50/50,  $M_w=2,000$ ), and 7.2 grams of the urea formaldehyde, and more specifically, the methylated urea resin CYMEL® U-65 (obtained from CYTEC Industries, Inc., viscosity 3,800 to 5,600 mPa·s at 25° C.) in a solvent mixture of xylene and 1-butanol (50/50 mixture), and with a total solid content of about 48 percent in an attritor mill with about 0.4 to about 0.6 millimeter size  $ZrO_2$  beads for 6.5 hours, and then filtering with a 20 micron Nylon filter. A 30 millimeter aluminum drum substrate was then coated with the aforementioned generated dispersion using known coating techniques as illustrated herein. After drying at 160° C. for 20 minutes, a hole blocking layer of  $TiO_2$  in the above phenolic formaldehyde resin and urea formaldehyde resin ( $TiO_2$ /phenolic formaldehyde resin/urea formaldehyde resin, ratio was 60/16/24) about 6 microns in thickness was obtained.

#### Example II

A photoconductor is prepared by repeating the above process of Comparative Example 1, except that the hole blocking layer dispersion is prepared by milling 18 grams of  $TiO_2$  (MT-150W, manufactured by Tayca Co., Japan), 9.6 grams of the phenolic formaldehyde resin VARCUMTM 29159 (obtained from OxyChem Company, about 50 percent in xylene/1-butanol=50/50,  $M_w=2,000$ ), and 7.2 grams of the urea formaldehyde resin a butylated urea resin CYMEL® U-80 (obtained from CYTEC Industries, Inc., viscosity 1,200 to 3,400 mPa·s at 25° C.) in a solvent mixture of xylene and 1-butanol (50/50 mixture), and with a total solid content of about 48 percent in an attritor mill with about 0.4 to about 0.6 millimeter size  $ZrO_2$  beads for 6.5 hours, and then filtering with a 20 micron Nylon filter. A 30 millimeter aluminum drum substrate is then coated with the aforementioned gen-

20

erated dispersion using known coating techniques as illustrated herein. After drying at 160° C. for 20 minutes, a hole blocking layer of  $TiO_2$  in the above phenolic formaldehyde resin and urea formaldehyde resin ( $TiO_2$ /phenolic formaldehyde resin/urea formaldehyde resin, ratio was 60/16/24) about 6 microns in thickness is obtained.

#### Example III

10 A photoconductor is prepared by repeating the above process of Comparative Example 1, except that the hole blocking layer dispersion is prepared by milling 18 grams of  $TiO_2$  (MT-150W, manufactured by Tayca Co., Japan), 9.6 grams of the phenolic formaldehyde resin VARCUMTM 29159 (obtained from OxyChem Company, about 50 percent in xylene/1-butanol=50/50,  $M_w=2,000$ ), and 12 grams of the urea formaldehyde, and more specifically, the isobutylated urea resin CYMEL® U-662 (obtained from CYTEC Industries, Inc., about 60 percent in xylene/1-butanol=50/50, viscosity 1,000 to 2,000 mPa·s at 25° C.,  $M_w=4,000$ ) in a solvent mixture of xylene and 1-butanol (50/50 mixture), and with a total solid content of about 48 percent in an attritor mill with about 0.4 to about 0.6 millimeter size  $ZrO_2$  beads for 6.5 hours, and then filtering with a 20 micron Nylon filter. A 30 millimeter aluminum drum substrate is then coated with the aforementioned generated dispersion using known coating techniques as illustrated herein. After drying at 160° C. for 20 minutes, a hole blocking layer of  $TiO_2$  in the above phenolic formaldehyde resin and urea formaldehyde resin ( $TiO_2$ /phenolic formaldehyde resin/urea formaldehyde resin, ratio was 60/16/24) about 6 microns in thickness is obtained.

#### Electrical Property Testing

35 The above prepared photoconductors of Comparative Example 1 and Example I were tested in a scanner set to obtain photoinduced discharge cycles, sequenced at one charge-erase cycle followed by one charge-expose-erase cycle, wherein the light intensity was incrementally increased 40 with cycling to produce a series of photoinduced discharge characteristic (PIDC) curves from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. These four photoconductors were tested at surface potentials of 700 volts with the exposure light intensity incrementally 45 increased by regulating a series of neutral density filters; the exposure light source was a 780 nanometer light emitting diode. The xerographic simulation was completed in an environmentally controlled light tight chamber at dry conditions (10 percent relative humidity and 22° C.).

50 55 The above prepared photoconductors exhibited substantially similar PIDCs. Thus, incorporation of the resin mixture of Example I in the hole blocking or undercoat layer did not adversely affect the electrical properties of the photoconductor.

60

#### Ghosting Measurement

The Comparative Example 1 and Example I photoconductor were acclimated at room temperature for 24 hours before 65 testing in A zone (85° F. and 80 percent humidity) for A zone ghosting. Print testing was accomplished in the Xerox Corporation WorkCentreTM Pro C3545 using the K (black toner)

station at  $t$  of 500 print counts ( $t$  equal to 0 is the first print;  $t$  equal to 500 is the 500<sup>th</sup> print). At the CMY stations of the color WorkCentre™ Pro C3545, run-up from  $t$  of 0 to  $t$  of 500 print counts for the photoconductor was completed. The prints for determining ghosting characteristics includes an X symbol or letter on a half tone image. When X is invisible, the ghost level is assigned Grade 0; when X is barely visible, the ghost level is assigned Grade 1; Grade 2 to Grade 5 refers to the level of visibility of X with Grade 5 meaning a dark and visible X. Ghosting levels were visually measured against an empirical scale, the smaller the ghosting grade (absolute value), the better the print quality. A negative ghosting grade number, such as -1, translates into an improved ghosting with regard to Comparative Example 1. The ghosting results in A zone are summarized in Table 1.

TABLE 1

| Photoconductors in A Zone                                | Ghosting Grade at $t$ of 0 | Ghosting Grade at $t$ of 500 prints |
|----------------------------------------------------------|----------------------------|-------------------------------------|
| Comparative Example 1, $TiO_2$ /Phenolic Resin = 60/40   | Grade -3                   | Grade -4                            |
| Example I, $TiO_2$ /Phenolic Resin/Urea Resin = 60/16/24 | Grade 0                    | Grade -1                            |

In A zone and at  $t=0$ , the ghosting level for the Example I photoconductor was low and excellent at Grade 0; in contrast, the Comparative Example 1 photoconductor had an elevated poor ghosting level of Grade -3. After 500 prints, the ghosting level for the Example I photoconductor remained low at Grade -1; in contrast, the Comparative Example 1 photoconductor had an elevated ghosting level of Grade -4. The disclosed hole blocking layer comprised of the phenolic resin/urea resin mixture exhibited almost no ghosting or very low ghosting in A zone; in contrast, the Comparative hole blocking layer comprised of the phenolic resin exhibited high ghosting.

Similarly, the Comparative Example 1 and Example I photoconductor were acclimated at room temperature for 24 hours before testing in J zone (25° F. and 10 percent humidity) for J zone ghosting. The ghosting results in J zone are summarized in Table 2.

TABLE 2

| Photoconductors in J zone                                | Ghosting Grade at $t$ of 0 | Ghosting Grade at $t$ of 500 prints |
|----------------------------------------------------------|----------------------------|-------------------------------------|
| Comparative Example 1, $TiO_2$ /Phenolic Resin = 60/40   | Grade -4                   | Grade -5                            |
| Example I, $TiO_2$ /Phenolic Resin/Urea Resin = 60/16/24 | Grade -1                   | Grade -2                            |

In J zone and at  $t=0$ , (time equals zero) the ghosting level for the Example I photoconductor was an excellent and improved low at Grade -1; in contrast, the Comparative Example 1 photoconductor had an elevated poor ghosting level of Grade -4. After 500 prints, the ghosting level for the Example I photoconductor remained low at Grade -2; in contrast, the Comparative Example 1 photoconductor had an elevated very poor ghosting level of Grade -5. The disclosed hole blocking layer comprised of the phenolic resin/urea resin mixture exhibited very low ghosting in J zone; in contrast, the Comparative hole blocking layer comprised of the phenolic resin exhibited high unacceptable ghosting.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, 10 position, size, shape, angle, color, or material.

What is claimed is:

1. A photoconductor consisting of and in sequence a supporting substrate, a ground plane layer, an undercoat layer thereover consisting of a crosslinked interpolymer network mixture of a metal oxide, a urea formaldehyde resin and a phenolic formaldehyde resin; a photogenerating layer, and a hole transport layer; wherein the phenolic formaldehyde resin is selected from the group consisting of a phenol, p-tert-butylphenol and cresol formaldehyde resin, a 4,4'-(1-methyl-20 ethylidene)bisphenol formaldehyde resin, a phenol and cresol formaldehyde resin, or a phenol and p-tert-butylphenol formaldehyde resin; the metal oxide is selected from the group consisting of titanium oxide, zinc oxide, tin oxide, aluminum oxide, silicone oxide, zirconium oxide, indium oxide, and molybdenum oxide; the photogenerating layer consists of a pigment and a resin binder; the hole transport layer consists of aryl amine molecules and a resin binder; and wherein the crosslinking value is from about 40 to about 90 percent, and wherein the urea formaldehyde resin consists of a methylated urea formaldehyde resin, an n-butylated urea formaldehyde resin or an isobutylated urea formaldehyde resin.

2. A photoconductor in accordance with claim 1 wherein said hole transport layer aryl amine molecules consists of at least one of



**23**

wherein X, Y, and Z are independently selected from the group consisting of alkyl, alkoxy, aryl, halogen, and mixtures thereof.

**3.** A photoconductor in accordance with claim **1** wherein said photogenerating layer pigment consists of at least one of a titanyl phthalocyanine, a hydroxygallium phthalocyanine, a halogallium phthalocyanine, a bisperylene, and mixtures thereof.

**4.** A photoconductor in accordance with claim **1** wherein said photogenerating layer is situated between said substrate and said hole transport layer consists of N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-

**24**

dimethylphenyl)-[p-terphenyl]-4,4'-diamine, and N,N'-diphenyl-N,N'-bis(3-chlorophenyl)-[p-terphenyl]-4,4'-diamine.

**5.** A photoconductor in accordance with claim **1** wherein said ground plane is gold.

**6.** A photoconductor in accordance with claim **1**, wherein said ground plane is a gold containing compound.

**7.** A photoconductor in accordance with claim **1** wherein said urea formaldehyde resin is a methylated urea formaldehyde resin.

**8.** A photoconductor in accordance with claim **1** wherein said urea formaldehyde is an n-butylated urea, formaldehyde resin.

**9.** A photoconductor in accordance with claim **1** wherein said urea formaldehyde is an isobutylated urea formaldehyde resin.

**10.** A photoconductor in accordance with claim **1** wherein said met oxide a titanium oxide.

\* \* \* \* \*